

## UNITED STATES PATENT OFFICE

1,996,568

## BASE METAL FOR VITREOUS ENAMEL

Clarence H. Butts, Monroe, Mich., assignor to  
The Newton Steel Company, Monroe, Mich., a  
corporation of Ohio

No Drawing. Application July 11, 1932,  
Serial No. 622,019

2 Claims. (Cl. 148—21.5)

This invention relates, as indicated, to base metal for vitreous enamel and more particularly, to sheet steel adapted to receive a coating of vitreous enamel and when so coated, be employed 5 as a unit of construction in which enameled sheet metal articles are usually employed.

In manufacturing vitreous enameled sheet metal, two main difficulties, from the standpoint of the present invention, have been encountered 10 in the past, i. e., first, the tendency of the sheet metal to give off occluded gases during the firing operation and second, the tendency of the sheet metal blanks to warp or sag and otherwise lose their shape during the firing operation.

15 As is well known to those familiar with the art, vitreous enamel finishes are usually produced by applying what is commonly termed a ground coat to a suitable metallic base, firing such ground coat and then applying either one or 20 more finish coats and then firing such finish coats.

For a number of reasons which need not be gone into at this time, the above referred to ground coat is usually dark in color, in the most 25 instances, a very dark blue which is nearly black. The finished coats, however, are usually light in color, the majority being pure white.

The occurrence of minute dark colored specks has been observed in the production of a large 30 percentage of light colored vitreous enamel finishes. It has been found that these dark specks are due to gases which are given up by the base metal during the firing of the finish coat, such gas bubbling through the ground coat and causing 35 a small quantity of such ground coat to be driven through the finish coat to produce these dark specks.

As above indicated, another principal difficulty 40 encountered in the manufacture of vitreous enamel finished sheet metal articles, especially when such articles are formed into unusual shapes, is the tendency of the metal blank to warp or sag out of shape during the firing of the vitreous enamel finish. If the warping is considerable, the blank must be scrapped for the 45 reason that a distortion of the blank after the enamel has been fired will cause the occurrence of hair cracks and like imperfections when fabricated.

50 It is among the objects of my invention to provide a base metal for vitreous enamel finishes which shall have none of the above named undesirable characteristics. Other objects of my invention will appear as the description proceeds.

55 For purposes of convenience, a formula giving

the range of percentages of the different important ingredients in the steel previously employed as a base metal for enamel finishes is reproduced below:

|                      |                  |      |   |
|----------------------|------------------|------|---|
| Sulphur              | .025 to          | .040 | 5 |
| Phosphorus           | .004 to          | .020 |   |
| Carbon               | .012 to          | .030 |   |
| Manganese            | .030 to          | .080 |   |
| Silicon              | Trace            |      |   |
| Iron (by difference) | 99.929 to 99.830 | 10   |   |

The process comprising my invention for producing a non-bubbling and non-warping base metal comprises refining the metal in the furnace to a point where the carbon content is under 15 .025% and the manganese content is under .060%. After the metal has been so refined, the proper amount of deoxidizing agents, i. e., manganese and silicon, are added so that the essential ingredients in the resultant metal will analyze as 20 follows:

|                      |                  |      |    |
|----------------------|------------------|------|----|
| Sulphur              | .025 to          | .040 |    |
| Phosphorus           | .004 to          | .020 |    |
| Carbon               | .012 to          | .060 | 25 |
| Manganese            | .040 to          | .300 |    |
| Silicon              | .030 to          | .100 |    |
| Iron (by difference) | 99.889 to 99.480 |      |    |

In the above table the range of silicon content has been given as between .030 and .100 and steel 30 containing this range of silicon has been found satisfactory for the above defined results, however, optimum results are obtained when the silicon range is from .060 to .080.

In addition to the above there may be added 35 to the metal a small quantity, i. e., from one-half to two pounds, of aluminum or aluminum titanium per ton of metal depending upon the state of oxidation of the molten bath.

Metal having the above treatment and composition 40 has been found to be far superior to ordinary "killed" steel, for the reason that while ordinary "killed" steel may not appreciably bubble during the firing operation, in the vitreous enamel process, nevertheless, such "killed" steel is 45 subject to excessive warpage or sag; whereas, steel manufactured according to the process comprising my invention and when properly processed in sheet form, as presently to be described, 50 does not evolve occluded, gas during the firing operation and does not warp or sag an appreciable amount.

Ordinary silicon "killed" steels are very soft 55 at elevated temperatures and accordingly, do not retain their shape during the enameling process.

After the metal of the above referred to desirable composition and produced in the manner specified has been rolled into sheets, such sheets are box annealed at a temperature of 5 from 1200° Fahrenheit to 1500° Fahrenheit, such box annealing preferably being followed by normalizing or open annealing the sheets, if it is necessary, to produce the proper physical results. Normalization or open annealing will not prevent warpage or sag without first box annealing the sheets. So long as the sheets are box annealed, fairly good results may be secured by normalizing before box annealing. However, best results are obtained if the normalizing step 10 follows the box annealing.

The manner of producing the base metal and its composition, as above set forth, may be satisfactorily employed in vitreous enameling processes without appreciable bubbling and hence, a 20 light colored coat may be applied to a dark colored ground coat without the occurrence of objectional spots incidental to a bubbling action. The metal treated in the manner described also is characterized by the fact that it retains its 25 shape and does not warp or sag during the firing operation.

Other modes of applying the principle of my invention may be employed instead of the one explained, change being made as regards the 30 materials employed, provided the ingredients stated by any of the following claims or the equivalent of such stated ingredients be employed.

I therefore particularly point out and distinctly 35 claim as my invention:—

1. The process of manufacturing sheet steel

suitable for receiving a fired coat of vitreous enamel which includes the steps of refining the steel to a stage where the carbon content is below 0.025% and the manganese content is below 0.060%, then adding to the steel alloying elements in sufficient quantities so that the steel has substantially the following composition:

Sulphur from \_\_\_\_\_ 0.025% to 0.040%  
 Phosphorus from \_\_\_\_\_ .004% to .020%  
 Carbon from \_\_\_\_\_ .012% to .060%  
 Manganese from \_\_\_\_\_ .040% to .300%  
 Silicon from \_\_\_\_\_ .030% to .100%

the remainder being substantially iron, rolling such metal to sheet form, and then box annealing 15 and normalizing such sheets.

2. The process of manufacturing sheet steel suitable for receiving a fired coat of vitreous enamel which includes the steps of refining the steel to a stage where the carbon content is below 20 0.025% and the manganese content is below 0.060%, then adding to the steel alloying elements in sufficient quantities so that the steel has substantially the following composition:

Sulphur from \_\_\_\_\_ 0.025% to 0.040%  
 Phosphorus from \_\_\_\_\_ .004% to .020%  
 Carbon from \_\_\_\_\_ .012% to .060%  
 Manganese from \_\_\_\_\_ .040% to .300%  
 Silicon from \_\_\_\_\_ .030% to .100%

the remainder being substantially iron, rolling such metal to sheet form, box annealing such sheets at a temperature from about 1200° F. to about 1500° F. and then normalizing such sheets.

CLARENCE H. BUTTS.

35